

Aug. 3, 1954

G. M. HAIST ET AL

2,685,514

DIRECT POSITIVE PHOTOGRAPHIC DEVELOPMENT PROCESS

Filed Aug. 3, 1953

CURVES A,B,C - NO QUATERNARY AMMONIUM  
COMPOUND IN DEVELOPER  
CURVES D,E,F - 3-METHYL-2-( $\beta$ -PHENETHYL-  
ISOQUINOLINIUM BROMIDE IN  
DEVELOPER



GRANT M. HAIST  
HAROLD D. RUSSELL  
INVENTORS

BY Daniel J. Mayne  
W. H. McJowell  
ATTORNEY & AGENT

## UNITED STATES PATENT OFFICE

2,685,514

## DIRECT POSITIVE PHOTOGRAPHIC DEVELOPMENT PROCESS

Grant M. Haist and Harold D. Russell, Rochester, N. Y., assignors to Eastman Kodak Company, Rochester, N. Y., a corporation of New Jersey

Application August 3, 1953, Serial No. 371,946

17 Claims. (Cl. 95—88)

1

This invention relates to a direct positive process for the development of photographs and particularly to methods for accelerating development in a direct positive process.

In the Ives U. S. Patent 2,563,785, August 7, 1951, and the Bean et al. U. S. Patent 2,604,400, July 22, 1952, is described a process for the development of direct positive images in an exposed internal latent image emulsion by use of developer compositions containing hydrazine or certain hydrazine derivatives.

We have found that the development activity of hydrazine-containing developers, particularly when they are used for the development of direct positive images in an exposed internal latent image emulsion, is appreciably accelerated and the useful life of the developer composition is materially extended, if certain quaternary ammonium compounds are incorporated into the hydrazine-containing developer.

The accompanying drawings illustrate the acceleration of development obtained by use of certain quaternary ammonium compounds in a developer composition for developing an internal latent image emulsion.

The effective quaternary ammonium compounds are as follows:

1.



3-methyl-2-β-phenethyl isoquinolinium bromide

2.



2-benzyl-3-methyl isoquinolinium bromide

3.



1-β-phenethyl β-picolinium bromide

4.



1-β-phenethyl quinolinium bromide

2



1-β-phenethyl lepidinium bromide

Many other quaternary ammonium compounds have been found not to be effective in accelerating development in the process of our invention; for example, the following:

- 15 2-methyl benzoselenazole methyl iodide  
Methyl benzotriazolium p-tolene sulfonate  
6-amino-benzothiazole dimethyl perchlorate  
1-benzyl-α-picolinium bromide  
1-benzyl-β-picolinium bromide  
20 1-benzyl-γ-picolinium bromide  
1-β-phenethyl-γ-picolinium bromide  
1-β-phenethyl quinaldinium bromide  
Dimethylene pyridinium perchlorate  
β-Phenylethyl-α-picolinium bromide  
25 p-Tert. butylphenoxyethoxy - ethyl - pyridinium perchlorate  
N,N' - ethylene - dioxyethyl pyridinium perchlorate

30 The photographic emulsion used in the process of our invention is a gelatino-silver halide emulsion such as a silver bromide emulsion, a silver bromoiodide emulsion or a silver chloro-iodide emulsion. It need not contain optical sensitizing dyes although certain sensitizing dyes may be added to it for the purpose of optical sensitizing or for promoting reversal. The emulsion should be undigested or if digested, the digestion should be carried out without the use of sulfur sensitizers. An emulsion of this type is that known as Burton's emulsion, described in Wall, "Photographic Emulsions," 1929, pages 52 and 53. Burton's emulsion is made as follows:

- 45 A. Silver nitrate ----- g. 100  
Water ----- cc. 500  
Ammonia—to form clear solution.
- B. Potassium bromide ----- g. 80  
Potassium iodide ----- g. 50  
Soft gelatin ----- g. 20  
50 Water ----- cc. 1,000  
C. Dry gelatin ----- g. 250

B is heated to 70° C. and A, cold, added to B with constant shaking, digested for 20 minutes at 50° C., and allowed to cool slowly. C is added

after being allowed to swell for 20 minutes in water, drained and melted. The emulsion is then set and washed.

An internal latent image emulsion, that is, one which forms the latent image mostly inside the silver halide grains, as described on pages 296 and 297 of Mess' "The Theory of the Photographic Process," 1942, is especially useful for the process of our invention.

Most of the internal latent image emulsions are silver bromoiodide emulsions of high iodide content, preferably containing at least 10%-20% of the halide as iodide. Burton's emulsion is an emulsion of this type, having a silver iodide content of approximately 40% of the content of 10 silver halide. It is not absolutely essential, however, for the emulsion to contain silver iodide.

An internal latent image emulsion made as described in Davey and Knott U. S. Patent No. 2,592,250, may also be used according to our invention. This emulsion is prepared by first forming in the absence of ammonia and in one or more stages, silver salt grains consisting at least partly of a silver salt which is more soluble in water than silver bromide, subsequently converting the grains to silver bromide or silver bromoiodide and if the silver iodide content of the emulsion is less than 6% calculated on the total silver halide, treating such grains with an iodine compound to bring the silver iodide up to at least 6%, ripening preferably in the absence of ammonia and then either washing out some of the soluble salts or washing out the whole of the soluble salts, followed by the addition of soluble salts such as soluble chloride or bromide. An example of an emulsion made in this way is as follows:

*Solution No. 1*

|               |         |           |
|---------------|---------|-----------|
| Inert gelatin | 20 g.   | at 40° C. |
| KCl           | 30 g.   |           |
| Water         | 560 cc. |           |

*Solution No. 2*

|       |         |           |
|-------|---------|-----------|
| KCl   | 100 g.  | at 45° C. |
| Water | 520 cc. |           |

*Solution No. 3*

|                   |         |           |
|-------------------|---------|-----------|
| AgNO <sub>3</sub> | 195 g.  | at 45° C. |
| Water             | 520 cc. |           |

*Solution No. 4*

|       |         |           |
|-------|---------|-----------|
| KBr   | 160 g.  | at 45° C. |
| KI    | 40 g.   |           |
| Water | 500 cc. |           |

Run Solutions Nos. 2 and 3 simultaneously into Solution No. 1 in a vessel, taking 90 seconds to do this. Then ripen for 1 minute at 45° C. Next add 235 grams of inert gelatin (dry). Then ripen at 45° C. for 15 minutes during which time the gelatin dissolves. Set and shred the emulsion and then wash until free from all soluble bromide and then add about 150 cc. of 10% solution of KCl (by weight), and then add water to make 3½ liters.

An internal latent image type of silver halide emulsion may be defined as one which, when a test portion is exposed to a light intensity scale for a fixed time between  $\frac{1}{100}$  and 1 second, and developed for 4 minutes at 20° C. in the ordinary "surface" developer (Example I), exhibits a maximum density not greater than  $\frac{1}{5}$  the maximum density obtained when the same emulsion is equally exposed and developed for 3 minutes at 20° C. in an internal type developer (Example II). Preferably the maximum density obtained

with the surface developer is not greater than  $\frac{1}{10}$  the maximum density obtained when the same emulsion is developed in the internal type developer. Stated conversely, an internal latent image emulsion, when developed in an internal type developer (Example II) exhibits a maximum density at least 5, and preferably at least 10, times the maximum density obtained when the same emulsion is exposed in the same way and developed in a surface developer (Example I).

Our process is carried out by exposing the internal latent image emulsion layer to an object or image and then placing the exposed emulsion layer directly in a silver halide developing solution containing one or more hydrazines such as those mentioned hereinafter and in addition, containing one or more of the above-mentioned effective quaternary ammonium compounds as well as developing agent. Alternately, the hydrazine can be incorporated into the internal latent image emulsion in which case the exposed emulsion layer is developed in a developer solution containing one or more of the mentioned effective quaternary ammonium compounds as well as a developing agent.

Developing agents suitable for use in the process of our invention include the usual phenolic or aminophenol type developing agents such as N-methyl-p-aminophenol sulfate, hydroquinone, 30 catechol, 2-methyl hydroquinone, 2-chlorohydroquinone, p-aminophenol, and pyrogallol. Also, 3-pyrazolidone developing agents are very useful in our developer compositions, for example, 1-(p-β-hydroxyethylphenyl)-3-pyrazolidone, 1-phenyl-3-pyrazolidone, 1-phenyl-2-acetyl-3-pyrazolidone, and particularly the 1-aryl-4,4-dialkyl-3-pyrazolidones such as 1-phenyl-4,4-dimethyl-3-pyrazolidone, 1-(p-β-hydroxyethylphenyl)-4,4-dimethyl-3-pyrazolidone and 1-p-tolyl-4,4-dimethyl-3-pyrazolidone described in Allen et al. U. S. patent application Serial No. 372,148 filed August 3, 1953, and in the Reynolds and Tinker U. S. patent application Serial No. 372,167, filed August 3, 1953.

Particularly efficacious developer compositions are those containing, in addition to the indicated effective quaternary ammonium compounds, a mixture of developing agents such as a mixture 50 of N-methyl-p-aminophenol and hydroquinone, or a mixture of hydroquinone and a 3-pyrazolidone developing agent.

The hydrazines useful in the developer compositions include those particularly described in the 55 Thirtle et al. U. S. Patent 2,618,656, November 18, 1952, and in the Weissberger U. S. patent application Serial No. 159,139 filed April 29, 1950, now Patent No. 2,663,732, such as the following:

|                                              |                                             |
|----------------------------------------------|---------------------------------------------|
| 60                                           | p-(Methylsulfonamidomethyl)-phenylhydrazine |
| m-(Methylsulfonamidomethyl)-phenylhydrazine  |                                             |
| o-(Methylsulfonamidomethyl)-phenylhydrazine  |                                             |
| p-(β-Methylsulfonamidoethyl)-phenylhydrazine |                                             |
| m-(β-Methylsulfonamidoethyl)-phenylhydrazine |                                             |
| o-(β-Methylsulfonamidoethyl)-phenylhydrazine |                                             |
| m-(Methylsulfonamido)-phenylhydrazine        |                                             |
| p-(Methylsulfonamido)-phenylhydrazine        |                                             |
| m-(Ethylsulfonamido)-phenylhydrazine         |                                             |
| p-(Ethylsulfonamido)-phenylhydrazine         |                                             |
| o-(Methylsulfonamido)-phenylhydrazine        |                                             |

The alkylsulfonamidoalkylphenylhydrazines and the alkylsulfonamidophenylhydrazines are particularly useful since they possess low toxicity characteristics compared to most of the other 75 hydrazines. In addition these hydrazines in

the presence of the quaternary ammonium compounds are much more effective in maintaining contrast than are other hydrazines such as phenyl hydrazine, nuclear-substituted phenylhydrazines and sulfonated naphthylhydrazines. The water-soluble salts of the hydrazines are, of course, very useful in preparing the developer compositions.

These hydrazines have the general formula:



in which D represents a divalent mononuclear arylene group of the benzene series, n represents a positive integer of from 1 to 5 and R represents an alkyl group of from 1 to 4 carbon atoms.

An ordinary surface type developer, that is, one which develops an image only on the surface of the grains of an internal latent image emulsion is the following:

*Example I*

|                             | G.  |
|-----------------------------|-----|
| p-Hydroxyphenylglycine      | 10  |
| Sodium carbonate (crystals) | 100 |
| Water to 1 liter.           |     |

Development time, 4 min. at 20° C.

An internal type developer, that is, one which develops an image inside the grains of an internal latent image emulsion is the following:

*Example II*

|                                | G. |
|--------------------------------|----|
| Hydroquinone                   | 15 |
| n-Methyl-p-aminophenol sulfate | 15 |
| Sodium sulfite (anhydrous)     | 50 |
| Potassium bromide              | 10 |
| Sodium hydroxide               | 25 |
| Sodium thiosulfate (crystals)  | 20 |
| Water to 1 liter.              |    |

Development time, 3 min. at 20° C.

Our invention will be further illustrated by reference to the following specific examples:

*Example III*

An emulsion made as described in the Davey and Knott application Serial No. 82,914 was coated on a support, dried and exposed on an intensity scale sensitometer to 3000° Kelvin tungsten illumination and developed for from 1 to 2 minutes at 75° F. in a solution of the following composition:

|                                                                     | G.         |
|---------------------------------------------------------------------|------------|
| N-methyl-p-aminophenol sulfate                                      | 5.0        |
| Hydroquinone                                                        | 10.0       |
| p-( <i>β</i> -Methylsulfonamidoethyl) phenylhydrazine hydrochloride | 2.0        |
| Sodium sulfite (desiccated)                                         | 75.0       |
| Trisodium phosphate, cryst.                                         | 75.0       |
| Diglycolic acid                                                     | 13.4       |
| 5-methyl benzotriazole                                              | 0.2        |
| Sodium hydroxide                                                    | 15.0       |
| 3-methyl-2- <i>β</i> -phenethylisoquinolinium bromide               | 0.4 to 0.6 |
| Water to make 1.0 liter.                                            |            |

A satisfactory direct positive image was obtained under these developing conditions and the developer compositions showed no adverse effects from oxidation.

The improvement in developing activity effected by use of the quaternary ammonium compound in this example is illustrated in the accompanying drawings wherein curves A, B and C show the appearance of the D-log E curves at different development times when development was conducted under the above conditions with the above

developer composition to which quaternary ammonium compound had been added. Curves D, E and F show that development was appreciably accelerated when it was carried out under the same conditions except for using the quaternary ammonium compound in the developer composition.

*Example IV*

10 A portion of the emulsion used in Example III was coated and exposed as in Example III and developed for 1 to 2 minutes at 75° F. in a solution of the following composition:

|                                                                        | G.   |
|------------------------------------------------------------------------|------|
| p - ( <i>β</i> - Methylsulfonamidoethyl) phenylhydrazine hydrochloride | 2.0  |
| Hydroquinone                                                           | 10.0 |
| 1-phenyl-3-pyrazolidone                                                | 0.5  |
| Sodium sulfite (desiccated)                                            | 75.0 |
| 5-methyl benzotriazole                                                 | 0.2  |
| 3-methyl-2- <i>β</i> -phenethylisoquinolinium bromide                  | 0.4  |
| Sodium hydroxide                                                       | 6.7  |
| Water to 1.0 liter.                                                    |      |

25 pH=11.5.

Under these development conditions a satisfactory direct positive image was obtained and the developer showed relatively little sign of oxidation.

*Example V*

30 A portion of the emulsion used in Example III was coated and exposed as in Example III and developed for 3 minutes at 75° F. in a solution of the following composition:

|                                                                        | G.   |
|------------------------------------------------------------------------|------|
| p - ( <i>β</i> - Methylsulfonamidoethyl) phenylhydrazine hydrochloride | 2.0  |
| Hydroquinone                                                           | 10.0 |
| n-Methyl-p-aminophenol sulfate                                         | 5.0  |
| Sodium sulfite (desiccated)                                            | 75.0 |
| Sodium carbonate monohydrate                                           | 40.0 |
| Benzotriazole                                                          | 0.2  |
| 3-methyl-2- <i>β</i> -phenethylisoquinolinium bromide                  | 0.2  |
| Water to make 1.0 liter.                                               |      |

45 pH=10.0.

Under these development conditions a satisfactory direct positive image was obtained and the developer showed no adverse signs of oxidation effects.

*Example VI*

50 A portion of the emulsion used in Example III was coated and exposed as in Example III and developed for 1 to 2 minutes at 75° F. in a solution of the following composition:

|                                                                     | G.   |
|---------------------------------------------------------------------|------|
| p-( <i>β</i> -Methylsulfonamidoethyl) phenylhydrazine hydrochloride | 2.0  |
| Hydroquinone                                                        | 10.0 |
| 1-phenyl-4,4-dimethyl-3-pyrazolidone                                | 1.0  |
| Sodium sulfite (desiccated)                                         | 75.0 |
| 5-methyl benzotriazole                                              | 0.2  |
| 3-methyl-2- <i>β</i> -phenethylisoquinolinium bromide               | 0.4  |
| Sodium hydroxide                                                    | 6.7  |
| Water to 1.0 liter.                                                 |      |

55 Under these development conditions a satisfactory direct positive image was obtained and the developer showed relatively little sign of oxidation.

## Example VII

A portion of the emulsion used in Example III was coated and exposed as in Example III and developed for 1 to 2 minutes at 75° F. in a solution of the following composition:

|                                                                    | G.   |    |
|--------------------------------------------------------------------|------|----|
| p-( $\beta$ -methylsulfonamidoethyl) phenylhydrazine hydrochloride | 2.0  |    |
| Hydroquinone                                                       | 10.0 | 10 |
| 1-(4'- $\beta$ -hydroxyethylphenyl) - 3 - pyrazolidone             | 1.0  |    |
| Sodium sulfite (desiccated)                                        | 75.0 |    |
| 5-methyl benzotriazole                                             | 0.2  |    |
| 3-methyl-2- $\beta$ -phenethylisoquinolinium bromide               | 0.4  |    |
| Sodium hydroxide                                                   | 6.7  |    |
| Water to 1.0 liter.                                                |      |    |
| ph=11.5.                                                           |      |    |

Under these development conditions a satisfactory direct positive image was obtained and the developer showed relatively little sign of oxidation.

An unexpected result of development, particularly by the methods of Examples IV, VI and VII, is that the developers remain cleaner and lighter in color and maintained their activity much longer than when the emulsion is developed with the same developer free of the quaternary ammonium compound. That is, the developers showed little coloration after several days intermittent use whereas the control developer turned red in a few hours, orange overnight and black in 3 days. It is to be further noted that superior keeping properties of the developers can be expected when the 3-pyrazolidone compounds are used in the developers in place of N-methyl-p-aminophenol.

It will be understood that the examples and modifications included herein are illustrative only and that our invention is to be taken as limited only by the scope of the appended claims.

What we claim is:

1. A photographic developing composition comprising an aqueous alkaline solution containing a mixture of a silver halide developing agent, a compound selected from the group consisting of 3-methyl-2- $\beta$ -phenethylisoquinolinium bromide, 2-benzyl-3-methylisoquinolinium bromide, 1- $\beta$ -phenethyl- $\beta$ -picolinium bromide, 1- $\beta$ -phenethylisoquinolinium bromide and 1- $\beta$ -phenethyl lepidinum bromide, and a hydrazine having the general formula



wherein D represents a divalent mononuclear arylene group of the benzene series, n represents a positive integer of from 1 to 5, and R represents an alkyl group of from 1 to 4 carbon atoms.

2. The photographic developer composition of claim 1 wherein the designated hydrazine has the general formula



wherein D represents a divalent mononuclear arylene group of the benzene series and R represents an alkyl group of from 1 to 4 carbon atoms.

3. The photographic developer composition of claim 1 wherein the designated developing agent is a 3-pyrazolidone silver halide developing agent.

4. The photographic developer composition of claim 1 wherein the designated hydrazine is p-( $\beta$ -methylsulfonamidoethyl)-phenylhydrazine.

5. A photographic developer composition comprising an aqueous alkaline solution containing

7 a mixture of a silver halide developing agent, 3-methyl-2- $\beta$ -phenethylisoquinolinium bromide, and a hydrazine having the general formula



wherein D represents a divalent mononuclear arylene group of the benzene series, n represents a positive integer of from 1 to 5, and R represents an alkyl group of from 1 to 4 carbon atoms.

6. A photographic developer composition comprising an aqueous alkaline solution containing a mixture of hydroquinone and N-methyl-p-aminophenol silver halide developing agents, p-( $\beta$ -methylsulfonamidoethyl) phenylhydrazine, and 3-methyl-2- $\beta$ -phenethylisoquinolinium bromide.

7. A photographic developer composition comprising an aqueous alkaline solution containing a mixture of hydroquinone and a 3-pyrazolidone silver halide developing agent, p-( $\beta$ -methylsulfonamidoethyl) phenylhydrazine, and 3-methyl-2- $\beta$ -phenethylisoquinolinium bromide.

20 8. A photographic developer composition comprising an aqueous alkaline solution containing a mixture of hydroquinone and 1-phenyl-3-pyrazolidone silver halide developing agents, p-( $\beta$ -methylsulfonamidoethyl) phenylhydrazine, and 3-methyl-2- $\beta$ -phenethylisoquinolinium bromide.

25 9. A photographic developer composition comprising an aqueous alkaline solution containing a mixture of hydroquinone and 1-phenyl-4,4-dimethyl-3-pyrazolidone silver halide developing agents, p-( $\beta$ -methylsulfonamidoethyl) phenylhydrazine, and 3-methyl-2- $\beta$ -phenethylisoquinolinium bromide.

30 35 10. A photographic developer composition comprising an aqueous alkaline solution containing a mixture of hydroquinone and 1-p-tolyl-4,4-dimethyl-3-pyrazolidone silver halide developing agents, p-( $\beta$ -methylsulfonamidoethyl) phenylhydrazine, and 3-methyl-2- $\beta$ -phenethylisoquinolinium bromide.

40 45 11. A photographic developer composition comprising an aqueous alkaline solution containing a mixture of a silver halide developing agent, 2-benzyl-3-methylisoquinolinium bromide, and a hydrazine having the general formula



50 where D represents a divalent mononuclear arylene group of the benzene series, n represents a positive integer of from 1 to 5, and R represents an alkyl group of from 1 to 4 carbon atoms.

55 12. A photographic developer composition comprising an aqueous alkaline solution containing a mixture of hydroquinone and N-methyl-p-aminophenol silver halide developing agents, p-( $\beta$ -methylsulfonamidoethyl) phenylhydrazine and 2-benzyl-3-methylisoquinolinium bromide.

60 13. A photographic developer composition comprising an aqueous alkaline solution containing a mixture of hydroquinone and a 3-pyrazolidone silver halide developing agent, p-( $\beta$ -methylsulfonamidoethyl) phenylhydrazine and 2-benzyl-3-methylisoquinolinium bromide.

65 14. A photographic developer composition comprising an aqueous alkaline solution containing a mixture of hydroquinone and 1-phenyl-3-pyrazolidone silver halide developing agents, p-( $\beta$ -methylsulfonamidoethyl) phenylhydrazine and 2-benzyl-3-methylisoquinolinium bromide.

70 15. A photographic developer composition comprising an aqueous alkaline solution containing a mixture of hydroquinone and 1-phenyl-4,4-dimethyl-3-pyrazolidone silver halide developing agents, p-( $\beta$ -methylsulfonamidoethyl) phen-

ylhydrazine and 2-benzyl-3-methylisoquinolinium bromide.

16. A photographic developer comprising an aqueous alkaline solution containing a mixture of hydroquinone and 1-p-tolyl-4,4-dimethyl-3-pyrazolidone silver halide developing agents, p-( $\beta$ -methylsulfonamidoethyl) phenylhydrazine and 2-benzyl-3-methylisoquinolinium bromide.

17. The method of obtaining a direct positive image in a silver halide emulsion layer which comprises exposing to light rays to which the emulsion is sensitive, a silver halide emulsion layer a test portion of which upon exposure to a light intensity scale for a fixed time between  $\frac{1}{100}$  and 1 second and development for 3 minutes at 20° C. in the following internal type developer (II):

|                                  | Grams |
|----------------------------------|-------|
| Hydroquinone                     | 15    |
| Monomethyl-p-aminophenol sulfate | 15    |
| Anhydrous sodium sulfite         | 50    |
| Potassium bromide                | 10    |
| Sodium hydroxide                 | 25    |
| Sodium thiosulfate               | 20    |
| Water to 1 liter.                | 25    |

gives a maximum density at least 5 times the

maximum density obtained when the equally exposed silver halide emulsion is developed for 4 minutes at 20° C. in the following surface developer (I):

|                        | Grams |
|------------------------|-------|
| p-Hydroxyphenylglycine | 10    |
| Sodium carbonate       | 100   |
| Water to 1 liter.      |       |

and developing only the unexposed portion of said emulsion layer in a developer containing a silver halide developing agent, a hydrazine having the general formula



wherein D represents a divalent mononuclear arylene group of the benzene series, n represents a positive integer of from 1 to 5, and R represents an alkyl group of from 1 to 4 carbon atoms, and a compound selected from the group consisting of 3-methyl-2- $\beta$ -phenethylisoquinolinium bromide, 2-benzyl-3-methylisoquinolinium bromide, 1- $\beta$ -phenethyl- $\beta$ -picolinium bromide, 1- $\beta$ -phenethylquinolinium bromide, and 1- $\beta$ -phenethyllepidinium bromide.

No references cited.